# EUROPEAN PATENT SPECIFICATION

(11) **EP 2 112 244 B1**
(45) Date of publication and mention of the grant of the patent: **01.05.2019**
(21) Application number: 09251028.8
(22) Date of filing: 31.03.2009
(51) Int. Cl.: C22C 21/10, C22F 1/053

(54) **METHOD OF FORMING HIGH STRENGTH L12 ALUMINIUM ALLOYS**
VERFAHREN ZUR HERSTELLUNG VON L12-ALUMINIUMLEGIERUNGEN MIT HOHER FESTIGKEIT
PROCÉDÉ DE FABRICATION D'ALLIAGES D'ALUMINIUM L12 À HAUTE RÉSISTANCE

(30) Priority: 18.04.2008 US 148387
(43) Date of publication of application: 28.10.2009
(73) Proprietor: United Technologies Corporation, Farmington, CT 06032 (US)
(72) Inventor: Pandey, Awadh B., Jupiter Florida 33458 (US)
(74) Representative: Dehns

(56) References cited:
- EP-A- 1 439 239
- WO-A-95/32074
- WO-A-96/10099
- WO-A-03/085145
- WO-A-03/085146
- WO-A-2004/046402
- CN-A- 1 436 870
- JP-A- 9 279 284
- US-A- 5 055 257
- US-A1- 2001 054 247
- US-A1- 2004 191 111
- US-A1- 2008 066 833
- RIDDLE, YANCY W. ET AL: "Recrystallization performance of AA7050 varied with Sc and Zr" MATERIALS SCIENCE FORUM , 331-337(PT. 2, ALLUMINIUM ALLOYS: THEIR PHYSICAL AND MECHANICAL PROPERTIES), 799-804 CODEN: MSFOEP; ISSN: 0255-5476, 2000, XP009117290
- MIL'MAN, YU. V. ET AL: "Effect of additional alloying with transition metals on the structure of an Al-7.1 Zn-1.3 Mg-0.12 Zr alloy" METALLOFIZIKA I NOVEISHIE TEKHNOLOGII , 26(10), 1363-1378 CODEN: MNTEEU; ISSN: 1024-1809, 2004, XP009117293

## Description

The present invention relates generally to aluminum alloys and more specifically to heat treatable aluminum alloys produced by melt processing and strengthened by L1₂ phase dispersions.

The combination of high strength, ductility, and fracture toughness, as well as low density, make aluminum alloys natural candidates for aerospace and space applications. However, their use is typically limited to temperatures below about 300°F (149°C) since most aluminum alloys start to lose strength in that temperature range as a result of coarsening of strengthening precipitates.

The development of aluminum alloys with improved elevated temperature mechanical properties is a continuing process. Some attempts have included aluminum-iron and aluminum-chromium based alloys such as Al-Fe-Ce, Al-Fe-V-Si, Al-Fe-Ce-W, and Al-Cr-Zr-Mn that contain incoherent dispersoids. These alloys, however, also lose strength at elevated temperatures due to particle coarsening. In addition, these alloys exhibit ductility and fracture toughness values lower than other commercially available aluminum alloys.

Other attempts have included the development of mechanically alloyed Al-Mg and Al-Ti alloys containing ceramic dispersoids. These alloys exhibit improved high temperature strength due to the particle dispersion, but the ductility and fracture toughness are not improved.

US-A-6,248,453 discloses aluminum alloys strengthened by dispersed Al₃X L1₂ intermetallic phases where X is selected from the group consisting of Sc, Er, Lu, Yb, Tm, and U. The Al₃X particles are coherent with the aluminum alloy matrix and are resistant to coarsening at elevated temperatures. The improved mechanical properties of the disclosed dispersion strengthened L1₂ aluminum alloys are stable up to 572°F (300°C). In order to create aluminum alloys containing fine dispersions of Al₃X L1₂ particles, the alloys need to be manufactured by expensive rapid solidification processes with cooling rates in excess of 1.8x10³ F/sec (10³ C/sec). US-A-2006/0269437 discloses an aluminum alloy that contains scandium and other elements. While the alloy is effective at high temperatures, it is not capable of being heat treated using a conventional age hardening mechanism.

WO95/32074, JP09279284, US2001/054247, US5055257, WO03/085146, WO03/085145, US2008/066833, WO2004/046402 Riddle, Yancy W. et al: "Recrystallization performance of AA7050 varied with Sc and Zr" Materials Science Forum, 331-337 799-804 and Mil'man, Yu V. et al: "Effect of additional alloying with transition metals on the structure of an Al-7.1 Zn-1.3 Mg-0.12 Zr alloy "Metallofizika I noveishie tekhnologii, 26(10), 1363-1378 all disclose aluminium alloys with zinc and magnesium. WO96/10099 discloses an aluminium alloy with the composition Al-7.0Z n - 1.5 Mg - 0.35 Sc-0.18 Zr-0.2 Ti.

Heat treatable aluminum alloys strengthened by coherent L1₂ intermetallic phases produced by standard, inexpensive melt processing techniques would be useful.

The present invention provides a method of forming a heat treatable aluminum alloy, the method comprising:
(a) forming a melt consisting of:
   5.0 to 9.0 weight percent zinc;
   1.5 to 3.0 weight percent magnesium;
   at least one first element selected from the group consisting of 0.1 to 0.5 weight percent scandium, 0.1 to 6.0 weight percent erbium, 0.1 to 10.0 weight percent thulium, 0.1 to 15.0 weight percent ytterbium, and 0.1 to 12.0 weight percent lutetium;
   at least one second element selected from the group consisting of 0.1 to 4.0 weight percent gadolinium, 0.1 to 4.0 weight percent yttrium, 0.05 to 1.0 weight percent zirconium, 0.05 to 2.0 weight percent titanium, 0.05 to 2.0 weight percent hafnium, and 0.05 to 1.0 weight percent niobium;
   optionally at least one of 0.001 weight percent to 0.1 weight percent sodium, 0.001 weight percent to 0.1 weight calcium, 0.001 weight percent to 0.1 weight percent strontium, 0.001 weight percent to 0.1 weight percent antimony, 0.001 weight percent to 0.1 weight percent barium and 0.001 weight percent to 0.1 weight percent phosphorus;
   optionally no more than 0.1 weight percent iron, 0.1 weight percent chromium, 0.1 weight percent manganese, 0.1 weight percent vanadium, 0.1 weight percent cobalt, and 0.1 weight percent nickel;
   and the balance being aluminum with unavoidable impurities;
(b) solidifying the melt to form a solid body; and
(c) heat treating the solid body;
   wherein the solidifying comprises a rapid solidification process in which the cooling rate is greater than 10³ °C/second; and
   wherein the heat treating comprises:
   solution heat treatment at 800°F (426°C) to 1100°F (593°C) for thirty minutes to four hours;
   quenching; and
   aging at 200°F (93°C) to 600°F (316°C) for two to forty-eight hours.

The present invention is a method to form heat treatable aluminum alloys by rapid solidification, and thereafter heat treated. The alloys can achieve high temperature performance and can be used at temperatures up to about 650°F (343°C).

These alloys comprise zinc, magnesium, and an Al₃X L1₂ dispersoid where X is at least one first element selected from scandium, erbium, thulium, ytterbium, and lutetium, and at least one second element selected from gadolinium, yttrium, zirconium, titanium, hafnium, and niobium.

Certain preferred embodiments of the present invention will now be described in greater detail by way of example only and with reference to the accompanying drawings, in which:
FIG. 1 is an aluminum zinc phase diagram;
FIG. 2 is an aluminum magnesium phase diagram;
FIG. 3 is an aluminum scandium phase diagram;
FIG. 4 is an aluminum erbium phase diagram;
FIG. 5 is an aluminum thulium phase diagram;
FIG. 6 is an aluminum ytterbium phase diagram; and
FIG. 7 is an aluminum lutetium phase diagram.

The alloys of this invention are based on the aluminum, zinc, magnesium system. The amount of zinc in these alloys ranges from about 5.0 to about 9.0 weight percent. The amount of magnesium in these alloys ranges from about 1.5 to about 3.0 weight percent.

The aluminum zinc phase diagram is shown in FIG. 1. The aluminum zinc binary system is a eutectic alloy system involving a monotectoid reaction and a miscibility gap in the solid state. There is a eutectic reaction at 94 weight percent zinc at 717.8°F (381°C). Zinc has maximum solid solubility of 83.1 weight percent in aluminum at 717.8°F (381°C) which can be extended by rapid solidification processing. The solubility of zinc in aluminum decreases with a decrease in temperature. Zinc provides significant amount of precipitation strengthening in aluminum by precipitation of fine second phases. The present invention is focused on hypoeutectic alloy composition ranges. Decomposition of the supersaturated solid solution of zinc in aluminum gives rise to spherical and ellipsoidal GP zones; precipitates with rhombohedral structure which are coherent with aluminum matrix and an incoherent (α'Al).

The aluminum magnesium phase diagram is shown in FIG. 2. The binary system is a eutectic alloy system with a eutectic reaction at 36 weight percent magnesium and 842°F (450°C). Magnesium has maximum solid solubility of 16 weight percent in aluminum at 842°F (450°C) which can extended further by rapid solidification processing. Magnesium provides substantial solid solution strengthening in aluminum. In addition, magnesium provides precipitation strengthening through precipitation of Zn₂Mg (η') phase.

The alloys of this invention contain aluminum solid solutions containing zinc and magnesium. These alloys also contain precipitates consisting of fine dispersions of Zn₂Mg (η') phase by decomposition of supersaturated solid solutions. In the solid solutions are dispersions of Al₃X having an L1₂ structure where X is at least one element selected from scandium, erbium, thulium, ytterbium, and lutetium and at least one element selected from gadolinium, yttrium, zirconium, titanium, hafnium, and niobium.

Exemplary aluminum alloys of this invention include, but are not limited to (in weight percent):
about Al-(5-9)Zn-(1.5-3)Mg-(0.1-0.25)Sc-(0.5-2.0)Gd;
about Al-(5-9)Zn-(1.5-3)Mg-(0.2-2)Er-(0.5-2.0)Gd;
about Al-(5-9)Zn-(1.5-3)Mg-(0.2-4)Tm-(0.5-2.0)Gd;
about Al-(5-9)Zn-(1.5-3)Mg-(0.2-4)Yb-(0.5-2.0)Gd;
about Al-(5-9)Zn-(1.5-3)Mg-(0.2-4)Lu-(0.5-2.0)Gd;
about Al-(5-9)Zn-(1.5-3)Mg-(0.1-0.25)Sc-(0.5-2.0)Y;
about Al-(5-9)Zn-(1.5-3)Mg-(0.2-2)Er-(0.5-2.0)Y;
about Al-(5-9)Zn-(1.5-3)Mg-(0.2-4)Tm-(0.5-2.0)Y;
about Al-(5-9)Zn-(1.5-3)Mg-(0.2-4)Yb-(0.5-2.0)Y;
about Al-(5-9)Zn-(1.5-3)Mg-(0.2-4)Lu-(0.5-2.0)Y;
about Al-(5-9)Zn-(1.5-3)Mg-(0.1-0.25)Sc-(0.1-0.5)Zr;
about Al-(5-9)Zn-(1.5-3)Mg-(0.2-2)Er-(0.1-0.5)Zr;
about Al-(5-9)Zn-(1.5-3)Mg-(0.2-4)Tm-(0.1-0.5)Zr;
about Al-(5-9)Zn-(1.5-3)Mg-(0.2-4)Yb-(0.1-0.5)Zr;
about Al-(5-9)Zn-(1.5-3)Mg-(0.2-4)Lu-(0.1-0.5)Zr;
about Al-(5-9)Zn-(1.5-3)Mg-(0.1-0.25)Sc-(0.1-0.5)Ti;
about Al-(5-9)Zn-(1.5-3)Mg-(0.2-2)Er-(0.1-0.5)Ti;
about Al-(5-9)Zn-(1.5-3)Mg-(0.2-4)Tm-(0.1-0.5)Ti;
about Al-(5-9)Zn-(1.5-3)Mg-(0.2-4)Yb-(0.1-0.5)Ti;
about Al-(5-9)Zn-(1.5-3)Mg-(0.2-4)-Lu-(0.1-0.5)Ti;
about Al-(5-9)Zn-(1.5-3)Mg-(0.1-0.25)Sc-(0.1-0.5)Hf;
about Al-(5-9)Zn-(1.5-3)Mg-(0.2-2)Er-(0.1-0.5)Hf;
about Al-(5-9)Zn-(1.5-3)Mg-(0.2-4)Tm-(0.1-0.5)Hf;
about Al-(5-9)Zn-(1.5-3)Mg-(0.2-4)Yb-(0.1-0.5)Hf;
about Al-(5-9)Zn-(1.5-3)Mg-(0.2-4)Lu-(0.1-0.5)Hf;
about Al-(5-9)Zn-(1.5-3)Mg-(0.1-0.25)Sc-(0.1-0.5)Nb;
about Al-(5-9)Zn-(1.5-3)Mg-(0.2-2)Er-(0.1-0.5)Nb;
about Al-(5-9)Zn-(1.5-3)Mg-(0.2-4)Tm-(0.1-0.5)Nb;
about Al-(5-9)Zn-(1.5-3)Mg-(0.2-4)Yb-(0.1-0.5)Nb;
about Al-(5-9)Zn-(1.5-3)Mg-(0.2-4)Lu-(0.1-0.5)Nb.

In the inventive aluminum based alloys disclosed herein, scandium, erbium, thulium, ytterbium, and lutetium are potent strengtheners that have low diffusivity and low solubility in aluminum. All these elements form equilibrium Al₃X intermetallic dispersoids where X is at least one of scandium, erbium, ytterbium, lutetium, that have an L1₂ structure that is an ordered face centered cubic structure with the X atoms located at the corners and aluminum atoms located on the cube faces of the unit cell.

Scandium forms Al₃Sc dispersoids that are fine and coherent with the aluminum matrix. Lattice parameters of aluminum and Al₃Sc are very close (0.405nm and 0.410nm respectively), indicating that there is minimal or no driving force for causing growth of the Al₃Sc dispersoids. This low interfacial energy makes the Al₃Sc dispersoids thermally stable and resistant to coarsening up to temperatures as high as about 840°F (450°C). In the alloys of this invention these Al₃Sc dispersoids are made stronger and more resistant to coarsening at elevated temperatures by adding suitable alloying elements such as gadolinium, yttrium, zirconium, titanium, hafnium, niobium, or combinations thereof, that enter Al₃Sc in solution.

Erbium forms Al₃Er dispersoids in the aluminum matrix that are fine and coherent with the aluminum matrix. The lattice parameters of aluminum and Al₃Er are close (0.405 nm and 0.417 nm respectively), indicating there is minimal driving force for causing growth of the Al₃Er dispersoids. This low interfacial energy makes the Al₃Er dispersoids thermally stable and resistant to coarsening up to temperatures as high as about 842°F (450°C). Addition of magnesium in solid solution in aluminum increases the lattice parameter of the aluminum matrix, and decreases the lattice parameter mismatch further increasing the resistance of the Al₃Er to coarsening. Additions of zinc in aluminum provide significant precipitation strengthening through precipitation of fine second phase Zn₂Mg (η'). In the alloys of this invention, these Al₃Er dispersoids are made stronger and more resistant to coarsening at elevated temperatures by adding suitable alloying elements such as gadolinium, yttrium, zirconium, titanium, hafnium, niobium, or combinations thereof that enter Al₃Er in solution.

Thulium forms metastable Al₃Tm dispersoids in the aluminum matrix that are fine and coherent with the aluminum matrix. The lattice parameters of aluminum and Al₃Tm are close (0.405 nm and 420 nm respectively), indicating there is minimal driving force for causing growth of the Al₃Tm dispersoids. This low interfacial energy makes the Al₃Tm dispersoids thermally stable and resistant to coarsening up to temperatures as high as about 842°F (450°C). Addition of magnesium in solid solution in aluminum increases the lattice parameter of the aluminum matrix and decreases the lattice parameter mismatch further increasing the resistance to coarsening of the dispersoid. Addition of zinc in aluminum provides significant precipitation strengthening through precipitation of fine second phase Zn₂Mg (η'). In the alloys of this invention these Al₃Tm dispersoids are made stronger and more resistant to coarsening at elevated temperatures by adding suitable alloying elements such as gadolinium, yttrium, zirconium, titanium, hafnium, niobium, or combinations thereof that enter Al₃Tm in solution.

Ytterbium forms Al₃Yb dispersoids in the aluminum matrix that are fine and coherent with the aluminum matrix. The lattice parameters of Al and Al₃Yb are close (0.405 nm and 0.420 nm respectively), indicating there is minimal driving force for causing growth of the Al₃Yb dispersoids. This low interfacial energy makes the Al₃Yb dispersoids thermally stable and resistant to coarsening up to temperatures as high as about 842°F (450°C). Addition of magnesium in solid solution in aluminum increases the lattice parameter of the aluminum matrix and decreases the lattice parameter mismatch further increasing the resistance to coarsening of the Al₃Yb. Addition of zinc in aluminum provides significant precipitation strengthening through precipitation of fine second phase Zn₂Mg (η'). In the alloys of this invention, these Al₃Yb dispersoids are made stronger and more resistant to coarsening at elevated temperatures by adding suitable alloying elements such as gadolinium, yttrium, zirconium, titanium, hafnium, niobium, or combinations thereof that enter Al₃Yb in solution.

Lutetium forms Al₃Lu dispersoids in the aluminum matrix that are fine and coherent with the aluminum matrix. The lattice parameters of Al and Al₃Lu are close (0.405 nm and 0.419 nm respectively), indicating there is minimal driving force for causing growth of the Al₃Lu dispersoids. This low interfacial energy makes the Al₃Lu dispersoids thermally stable and resistant to coarsening up to temperatures as high as about 842°F (450°C). Addition of magnesium in solid solution in aluminum increases the lattice parameter of the aluminum matrix and decreases the lattice parameter mismatch further increasing the resistance to coarsening of Al₃Lu. Addition of zinc in aluminum provides significant precipitation strengthening through precipitation of fine second phase Zn₂Mg (η'). In the alloys of this invention, these Al₃Lu dispersoids are made stronger and more resistant to coarsening at elevated temperatures by adding suitable alloying elements such as gadolinium, yttrium, zirconium, titanium, hafnium, niobium, or mixtures thereof that enter Al₃Lu in solution.

Gadolinium forms metastable Al₃Gd dispersoids in the aluminum matrix that are stable up to temperatures as high as about 842°F (450°C) due to their low diffusivity in aluminum. The Al₃Gd dispersoids have a D0₁₉ structure in the equilibrium condition. Despite its large atomic size, gadolinium has fairly high solubility in the Al₃X intermetallic dispersoids (where X is scandium, erbium, thulium, ytterbium or lutetium). Gadolinium can substitute for the X atoms in Al₃X intermetallic, thereby forming an ordered L1₂ phase which results in improved thermal and structural stability.

Yttrium forms metastable Al₃Y dispersoids in the aluminum matrix that have an L1₂ structure in the metastable condition and a D0₁₉ structure in the equilibrium condition. The metastable Al₃Y dispersoids have a low diffusion coefficient which makes them thermally stable and highly resistant to coarsening. Yttrium has a high solubility in the Al₃X intermetallic dispersoids allowing large amounts of yttrium to substitute for X in the Al₃X L1₂ dispersoids which results in improved thermal and structural stability.

Zirconium forms Al₃Zr dispersoids in the aluminum matrix that have an L1₂ structure in the metastable condition and D0₂₃ structure in the equilibrium condition. The metastable Al₃Zr dispersoids have a low diffusion coefficient which makes them thermally stable and highly resistant to coarsening. Zirconium has a high solubility in the Al₃X dispersoids allowing large amounts of zirconium to substitute for X in the Al₃X dispersoids, which results in improved thermal and structural stability.

Titanium forms Al₃Ti dispersoids in the aluminum matrix that have an L1₂ structure in the metastable condition and DO₂₂ structure in the equilibrium condition. The metastable Al₃Ti dispersoids have a low diffusion coefficient which makes them thermally stable and highly resistant to coarsening. Titanium has a high solubility in the Al₃X dispersoids allowing large amounts of titanium to substitute for X in the Al₃X dispersoids, which results in improved thermal and structural stability.

Hafnium forms metastable Al₃Hf dispersoids in the aluminum matrix that have an L1₂ structure in the metastable condition and a D0₂₃ structure in the equilibrium condition. The Al₃Hf dispersoids have a low diffusion coefficient, which makes them thermally stable and highly resistant to coarsening. Hafnium has a high solubility in the Al₃X dispersoids allowing large amounts of hafnium to substitute for scandium, erbium, thulium, ytterbium, and lutetium in the above mentioned Al₃X dispersoids, which results in stronger and more thermally stable dispersoids.

Niobium forms metastable Al₃Nb dispersoids in the aluminum matrix that have an L1₂ structure in the metastable condition and a D0₂₂ structure in the equilibrium condition. Niobium has a lower solubility in the Al₃X dispersoids than hafnium or yttrium, allowing relatively lower amounts of niobium than hafnium or yttrium to substitute for X in the Al₃X dispersoids. Nonetheless, niobium can be very effective in slowing down the coarsening kinetics of the Al₃X dispersoids because the Al₃Nb dispersoids are thermally stable. The substitution of niobium for X in the above mentioned Al₃X dispersoids results in stronger and more thermally stable dispersoids.

Al₃X L1₂ precipitates improve elevated temperature mechanical properties in aluminum alloys for two reasons. First, the precipitates are ordered intermetallic compounds. As a result, when the particles are sheared by glide dislocations during deformation, the dislocations separate into two partial dislocations separated by an anti-phase boundary on the glide plane. The energy to create the anti-phase boundary is the origin of the strengthening. Second, the cubic L1₂ crystal structure and lattice parameter of the precipitates are closely matched to the aluminum solid solution matrix. This results in a lattice coherency at the precipitate/matrix boundary that resists coarsening. The lack of an interphase boundary results in a low driving force for particle growth and resulting elevated temperature stability. Alloying elements in solid solution in the dispersed strengthening particles and in the aluminum matrix that tend to decrease the lattice mismatch between the matrix and particles will tend to increase the strengthening and elevated temperature stability of the alloy.

The alloys are based on aluminum zinc magnesium systems. Addition of magnesium in solid solution in aluminum increases the lattice parameter of the aluminum matrix and decreases the lattice parameter mismatch further increasing the resistance to coarsening of the L1₂ Al₃X phases where X is at least one element selected from scandium, erbium, thulium, ytterbium, and lutetium and at least on element selected from gadolinium, yttrium, zirconium, titanium, hafnium, and niobium. Addition of zinc in aluminum provides significant precipitation strengthening through precipitation of fine second phase Zn₂Mg (η'). The amount of zinc in these alloys ranges from about 5.0 to about 9.0 weight percent. The amount of magnesium in these alloys ranges from about 1.5 to about 3.0 weight percent.

The amount of scandium present in the alloys of this invention, if any, may vary from about 0.1 to about 0.5 weight percent, more preferably from about 0.1 to about 0.35 weight percent, and even more preferably from about 0.1 to about 0.25 weight percent. The Al-Sc phase diagram shown in FIG. 3 indicates a eutectic reaction at about 0.5 weight percent scandium at about 1219°F (659°C) resulting in a solid solution of scandium and aluminum and Al₃Sc dispersoids. Aluminum alloys with less than 0.5 weight percent scandium can be quenched from the melt to retain scandium in solid solution that may precipitate as dispersed L1₂ intermetallic Al₃Sc following an aging treatment. Alloys with scandium in excess of the eutectic composition (hypereutectic alloys) can only retain scandium in solid solution by rapid solidification processing (RSP) where cooling rates are in excess of about 10³°C/second. Alloys with scandium in excess of the eutectic composition cooled normally will have a microstructure consisting of relatively large Al₃Sc grains in a finally divided aluminum-Al₃Sc eutectic phase matrix.

The amount of erbium present in the alloys of this invention, if any, may vary from about 0.1 to about 6.0 weight percent, more preferably from about 0.1 to about 4.0 weight percent, and even more preferably from about 0.2 to about 2.0 weight percent. The Al-Er phase diagram shown in FIG. 4 indicates a eutectic reaction at about 6 weight percent erbium at about 1211°F (655°C). Aluminum alloys with less than about 6 weight percent erbium can be quenched from the melt to retain erbium in solid solutions that may precipitate as dispersed L1₂ intermetallic Al₃Er following an aging treatment. Alloys with erbium in excess of the eutectic composition can only retain erbium in solid solution by rapid solidification processing (RSP) where cooling rates are in excess of about 10³°C/second. Alloys with erbium in excess of the eutectic composition (hypereutectic alloys) cooled normally will have a microstructure consisting of relatively large Al₃Er dispersoids in a finely divided aluminum-Al₃Er eutectic phase matrix.

The amount of thulium present in the alloys of this invention, if any, may vary from about 0.1 to about 10.0 weight percent, more preferably from about 0.2 to about 6.0 weight percent, and even more preferably from about 0.2 to about 4.0 weight percent. The Al-Tm phase diagram shown in FIG. 5 indicates a eutectic reaction at about 10 weight percent thulium at about 1193°F (645°C). Thulium forms metastable Al₃Tm dispersoids in the aluminum matrix that have an L1₂ structure in the equilibrium condition. The Al₃Tm dispersoids have a low diffusion coefficient which makes them thermally stable and highly resistant to coarsening. Aluminum alloys with less than 10 weight percent thulium can be quenched from the melt to retain thulium in solid solution that may precipitate as dispersed metastable L1₂ intermetallic Al₃Tm following an aging treatment. Alloys with thulium in excess of the eutectic composition can only retain Tm in solid solution by rapid solidification processing (RSP) where cooling rates are in excess of about 10³°C/second.

The amount of ytterbium present in the alloys of this invention, if any, may vary from about 0.1 to about 15.0 weight percent, more preferably from about 0.2 to about 8.0 weight percent, and even more preferably from about 0.2 to about 4.0 weight percent. The Al-Yb phase diagram shown in FIG. 6 indicates a eutectic reaction at about 21 weight percent ytterbium at about 1157°F (625°C). Aluminum alloys with less than about 21 weight percent ytterbium can be quenched from the melt to retain ytterbium in solid solution that may precipitate as dispersed L1₂ intermetallic Al₃Yb following an aging treatment. Alloys with ytterbium in excess of the eutectic composition can only retain ytterbium in solid solution by rapid solidification processing (RSP) where cooling rates are in excess of about 10³°C/second. Alloys with ytterbium in excess of the eutectic composition cooled normally will have a microstructure consisting of relatively large Al₃Yb grains in a finally divided aluminum-Al₃Yb eutectic phase matrix.

The amount of lutetium present in the alloys of this invention, if any, may vary from about 0.1 to about 12.0 weight percent, more preferably from about 0.2 to about 8.0 weight percent, and even more preferably from about 0.2 to about 4.0 weight percent. The Al-Lu phase diagram shown in FIG. 7 indicates a eutectic reaction at about 11.7 weight percent Lu at about 1202°F (650°C). Aluminum alloys with less than about 11.7 weight percent lutetium can be quenched from the melt to retain Lu in solid solution that may precipitate as dispersed L1₂ intermetallic Al₃Lu following an aging treatment. Alloys with Lu in excess of the eutectic composition can only retain Lu in solid solution by rapid solidification processing (RSP) where cooling rates are in excess of about 10³°C/second. Alloys with lutetium in excess of the eutectic composition cooled normally will have a microstructure consisting of relatively large Al₃Lu grains in a finely divided aluminum-Al₃Lu eutectic phase matrix.

The amount of gadolinium present in the alloys of this invention, if any, may vary from about 0.1 to about 4 weight percent, more preferably from 0.2 to about 2 weight percent, and even more preferably from about 0.5 to about 2 weight percent.

The amount of yttrium present in the alloys of this invention, if any, may vary from about 0.1 to about 4 weight percent, more preferably from 0.2 to about 2 weight percent, and even more preferably from about 0.5 to about 2 weight percent.

The amount of zirconium present in the alloys of this invention, if any, may vary from about 0.05 to about 1 weight percent, more preferably from 0.1 to about 0.75 weight percent, and even more preferably from about 0.1 to about 0.5 weight percent.

The amount of titanium present in the alloys of this invention, if any, may vary from about 0.05 to about 2 weight percent, more preferably from 0.1 to about 1 weight percent, and even more preferably from about 0.1 to about 0.5 weight percent.

The amount of hafnium present in the alloys of this invention, if any, may vary from about 0.05 to about 2 weight percent, more preferably from 0.1 to about 1 weight percent, and even more preferably from about 0.1 to about 0.5 weight percent.

The amount of niobium present in the alloys of this invention, if any, may vary from about 0.05 to about 1 weight percent, more preferably from 0.1 to about 0.75 weight percent, and even more preferably from about 0.1 to about 0.5 weight percent.

In order to have the best properties for the alloys of this invention, it is desirable to limit the amount of other elements. Specific elements that should be reduced or eliminated include no more than about 0.1 weight percent iron, about 0.1 weight percent chromium, about 0.1 weight percent manganese, about 0.1 weight percent vanadium, about 0.1 weight percent cobalt, and about 0.1 weight percent nickel. The total quantity of additional elements should not exceed about 1% by weight, including the above listed impurities and other elements.

Other additions in the alloys of this invention may include at least one of about 0.001 weight percent to about 0.10 weight percent sodium, about 0.001 weight percent to about 0.10 weight calcium, about 0.001 weight percent to about 0.10 weight percent strontium, about 0.001 weight percent to about 0.10 weight percent antimony, about 0.001 weight percent to about 0.10 weight percent barium and about 0.001 weight percent to about 0.10 weight percent phosphorus. These are added to refine the microstructure of the eutectic phase and the primary magnesium or lithium morphology and size.

These aluminum alloys are made by rapid solidification processing. The rapid solidification process should have a cooling rate greater that about 10³°C/second including but not limited to powder processing, atomization, melt spinning, splat quenching, spray deposition, cold spray, plasma spray, laser melting and deposition, ball milling and cryomilling.

## Claims

1. A method of forming a heat treatable aluminum alloy, the method comprising:
(a) forming a melt consisting of:
5.0 to 9.0 weight percent zinc;
1.5 to 3.0 weight percent magnesium;
at least one first element selected from the group consisting of 0.1 to 0.5 weight percent scandium, 0.1 to 6.0 weight percent erbium, 0.1 to 10.0 weight percent thulium, 0.1 to 15.0 weight percent ytterbium, and 0.1 to 12.0 weight percent lutetium;
at least one second element selected from the group consisting of 0.1 to 4.0 weight percent gadolinium, 0.1 to 4.0 weight percent yttrium, 0.05 to 1.0 weight percent zirconium, 0.05 to 2.0 weight percent titanium, 0.05 to 2.0 weight percent hafnium, and 0.05 to 1.0 weight percent niobium;
optionally at least one of 0.001 weight percent to 0.1 weight percent sodium, 0.001 weight percent to 0.1 weight calcium, 0.001 weight percent to 0.1 weight percent strontium, 0.001 weight percent to 0.1 weight percent antimony, 0.001 weight percent to 0.1 weight percent barium and 0.001 weight percent to 0.1 weight percent phosphorus;
optionally no more than 0.1 weight percent iron, 0.1 weight percent chromium, 0.1 weight percent manganese, 0.1 weight percent vanadium, 0.1 weight percent cobalt, and 0.1 weight percent nickel;
and the balance being aluminum with unavoidable impurities;
(b) solidifying the melt to form a solid body; and
(c) heat treating the solid body;
wherein the solidifying comprises a rapid solidification process in which the cooling rate is greater than 10³ °C/second; and
wherein the heat treating comprises:
solution heat treatment at 800°F (426°C) to 1100°F (593°C) for thirty minutes to four hours;
quenching; and
aging at 200°F (93°C) to 600°F (316°C) for two to forty-eight hours.

2. The method as claimed in claim 1, wherein the solid body comprises an aluminum solid solution matrix containing a plurality of dispersed Al₃X second phases having L1₂ structures, wherein X includes at least one first element and at least one second element.

3. The method of claim 1 or 2, further comprising:
refining the structure of the solid body by deformation processing comprising at least one of: extrusion, forging and rolling.

## Patentansprüche

1. Verfahren zur Herstellung einer wärmebehandelbaren Aluminiumlegierung, wobei das Verfahren Folgendes umfasst:
(a) Herstellen einer Schmelze, bestehend aus:
5,0 bis 9,0 Gewichtsprozent Zink;
1,5 bis 3,0 Gewichtsprozent Magnesium;
zumindest einem ersten Element, das aus der Gruppe ausgewählt ist, die aus 0,1 bis 0,5 Gewichtsprozent Scandium, 0,1 bis 6,0 Gewichtsprozent Erbium, 0,1 bis 10,0 Gewichtsprozent Thulium, 0,1 bis 15,0 Gewichtsprozent Ytterbium und 0,1 bis 12,0 Gewichtsprozent Lutetium besteht;
zumindest einem zweiten Element, das aus der Gruppe ausgewählt ist, die aus 0,1 bis 4,0 Gewichtsprozent Gadolinium, 0,1 bis 4,0 Gewichtsprozent Yttrium, 0,05 bis 1,0 Gewichtsprozent Zirkonium, 0,05 bis 2,0 Gewichtsprozent Titan, 0,05 bis 2,0 Gewichtsprozent Hafnium und 0,05 bis 1,0 Gewichtsprozent Niob besteht;
optional zumindest einem von 0,001 Gewichtsprozent bis 0,1 Gewichtsprozent Natrium, 0,001 Gewichtsprozent bis 0,1 Gewichtsprozent Calcium, 0,001 Gewichtsprozent bis 0,1 Gewichtsprozent Strontium, 0,001 Gewichtsprozent bis 0,1 Gewichtsprozent Antimon, 0,001 Gewichtsprozent bis 0,1 Gewichtsprozent Barium und 0,001 Gewichtsprozent bis 0,1 Gewichtsprozent Phosphor;
optional nicht mehr als 0,1 Gewichtsprozent Eisen, 0,1 Gewichtsprozent Chrom, 0,1 Gewichtsprozent Mangan, 0,1 Gewichtsprozent Vanadium, 0,1 Gewichtsprozent Kobalt und 0,1 Gewichtsprozent Nickel;
und wobei der Rest Aluminium mit unvermeidbaren Unreinheiten ist;
(b) Verfestigen der Schmelzen, um einen festen Körper herzustellen; und
(c) Wärmebehandeln des festen Körpers;
wobei das Verfestigen einen schnellen Verfestigungsvorgang umfasst, bei dem die Kühlrate größer als 10³ °C/Sekunde ist; und
wobei das Wärmebehandeln Folgendes umfasst:
Lösungswärmebehandlung bei 800 °F (426 °C) bis 1100 °F (593 °C) über dreißig Minuten bis vier Stunden;
Abschrecken; und
Altern bei 200 °F (93 °C) bis 600 °F (316 °C) über zwei bis achtundvierzig Stunden.

2. Verfahren nach Anspruch 1, wobei der feste Körper eine feste Aluminiumlösungsmatrix umfasst, die eine Vielzahl von dispergierten zweiten Al₃X-Phasen enthält, die L1₂-Strukturen aufweisen, wobei X zumindest ein erstes Element und zumindest ein zweites Element beinhaltet.

3. Verfahren nach Anspruch 1 oder 2, ferner umfassend:
Verfeinern der Struktur des festen Körpers durch Verformungsverarbeitung, umfassend zumindest eines von: Extrusion, Schmieden und Walzen.

## Revendications

1. Procédé de formation d'un alliage d'aluminium traitable thermiquement, le procédé comprenant :
(a) la formation d'un métal liquide constitué par :
5,0 à 9,0 pour cent en poids de zinc ;
1,5 à 3,0 pour cent en poids de magnésium ;
au moins un premier élément sélectionné à partir du groupe constitué par 0,1 à 0,5 pour cent en poids de scandium, 0,1 à 6,0 pour cent en poids d'erbium, 0,1 à 10,0 pour cent en poids de thulium, 0,1 à 15,0 pour cent en poids d'ytterbium, et 0,1 à 12,0 pour cent de lutétium ;
au moins un second élément sélectionné à partir du groupe constitué par 0,1 à 4,0 pour cent en poids de gadolinium, 0,1 à 4,0 pour cent en poids d'yttrium, 0,05 à 1,0 pour cent en poids de zirconium, 0,05 à 2,0 pour cent en poids de titane, 0,05 à 2,0 pour cent en poids d'hafnium, et 0,05 à 1,0 pour cent en poids de niobium ;
facultativement au moins l'un parmi 0,001 pour cent en poids à 0,1 pour cent en poids de sodium, 0,001 pour cent en poids à 0,1 pour cent en poids de calcium, 0,001 pour cent en poids à 0,1 pour cent en poids de strontium, 0,001 pour cent en poids à 0,1 pour cent en poids d'antimoine, 0,001 pour cent en poids à 0,1 pour cent en poids de baryum et 0,001 pour cent en poids à 0,1 pour cent en poids de phosphore ;
facultativement pas plus de 0,1 pour cent en poids de fer, 0,1 pour cent en poids de chrome, 0,1 pour cent en poids de manganèse, 0,1 pour cent en poids de vanadium, 0,1 pour cent en poids de cobalt, et 0,1 pour cent en poids de nickel ;
et le reste étant de l'aluminium avec des impuretés inévitables ;
(b) la solidification du métal liquide pour former un corps solide ; et
(c) le traitement thermique du corps solide ;
dans lequel la solidification comprend un processus de solidification rapide dans lequel le taux de refroidissement est supérieur à 10³ °C/seconde ; et
dans lequel le traitement thermique comprend :
un traitement thermique de la solution de 800 °F (426 °C) à 1 100 °F (593 °C) pendant trente minutes à quatre heures ;
une trempe ; et
un vieillissement de 200 °F (93 °C) à 600 °F (316 °C) pendant quarante-huit heures.

2. Procédé selon la revendication 1, dans lequel le corps solide comprend une matrice de solution solide d'aluminium contenant une pluralité de secondes phases d'Al₃X dispersées ayant des structures L1₂, dans lequel X inclut au moins un premier élément et au moins un second élément.

3. Procédé selon la revendication 1 ou 2, comprenant en outre :
l'affinement de la structure du corps solide par un processus de déformation comprenant au moins l'un parmi : l'extrusion, le forgeage et le laminage.
